

## UNITED STATES PATENT OFFICE

2,604,449

GREASES AND COMPOUNDS FOR MAKING  
SAME AND OTHER COMPOSITIONS

William C. Bryant, Garfield, and Anthony Giordano, Hackensack, N. J., assignors to Swan-Finch Oil Corporation, New York, N. Y., a corporation of New York

No Drawing. Application March 8, 1949,  
Serial No. 80,328

14 Claims. (Cl. 252—33.6)

1

This invention relates to greases and other compounds prepared from amic acids and salts of same. It also relates to such amic acids and derivatives thereof, including such salts.

Ordinary lubricating greases as now commercially produced are made by the addition of soap or a mixture of soaps to lubricating oils and/or other petroleum fractions. The soap or soaps serve to produce gelation of the mixture. The gelled mass may vary in consistency from a solid brick to a viscous oil of a slightly greater viscosity than the original oil. The usual greases are made up of calcium or soda or calcium and soda soaps in petroleum oil or other petroleum substance. Instead of soda, potassium or lithium soaps may be used alone or in combination with calcium, barium or strontium soaps. These calcium, soda and potassium greases have well-known disadvantages. For example, when using sodium or potassium soaps, the resultant greases are not resistant to water and, where used in wet places, form emulsions which run off the parts being lubricated. The lime soap grease and the soda and potassium soap greases have poor operating qualities at low temperature, each producing high starting torques at such low temperatures, for example, at  $-20^{\circ}$  F. On the other hand, when the calcium greases are heated up to the melting point, the water of gelation, the so-called "tie" water, is boiled off if the temperature remains at such point for any considerable time. Thereafter, when the grease cools, the soap tends to separate from the oil since it lacks the "tie" water. When the sodium and potassium greases are heated up and cooled, they tend to set to a much heavier mass which is unstable to shearing forces. The calcium greases, furthermore, have relatively low dropping points. Calcium and sodium and potassium greases have little rust preventive action. The barium and strontium greases require at least half again as much soap per equivalent gelling efficiency as the sodium greases. Barium and strontium greases are water resistant and resist temperatures up to about  $275^{\circ}$  F., but gradually harden so as to lose their efficiency as lubricants. The ordinary lithium greases have resistance to water but they do not function satisfactorily in applications where ambient temperatures exceed  $350^{\circ}$  F.

In addition, all of the greases heretofore made and mentioned above or proposed, except that in the copending application of Bryant and Frost, Serial No. 37,534, filed July 8, 1948, now Patent No. 2,594,286, have the disadvantage that they are made from fats and fatty acids which have con-

siderable variation in their constitution as procurable on the market from time to time and hence cause considerable variation in the greases produced therefrom.

The principal object of the present invention, accordingly, is to produce greases and other compounds prepared from salts of amic acids which shall overcome at least some of these disadvantages and which shall have superior characteristics to those found in the hitherto known greases mentioned above. Another object of the invention is to provide a suitable base for producing such greases. Another object of the invention is to provide a series of new and useful compounds consisting of amic acids, derivatives and compounds thereof.

The invention accordingly comprises the novel products, the specific embodiments of which are described hereinafter by way of example and in accordance with which we now prefer to practice the invention.

We have found in accordance with our invention that a composition containing a proportion of an alkali metal salt or a polyvalent metal salt of amic acid having the formula



where  $R_1$  is selected from the group consisting of methylene groups having a carbon chain length of 1 to 8 carbon atoms and the group



$R_2$  is an aliphatic radical of a carbon chain length of 4 to 18 carbon atoms, and  $R_3$  is selected from the group consisting of hydrogen and an aliphatic radical of a carbon chain length of 4 to 18 carbon atoms, mixed with a proportion of petroleum substance such as various petroleum oils, petrolatum or like substances, produces useful lubricating characteristics. When the salt of amic acid (or grease base) given in the formula is present in the proportion of about 6 to about 17% of the grease, it forms a smooth, semi-solid mass at room temperature. Compounds containing more than 17% range upwardly to an extremely hard consistency. The salt of amic acid (or grease base) may be contained in other proportions, say, from 0.5% to 30% of the composition for varying purposes. With 0.5% composition using a fluid petroleum oil such as cylinder oil, the composition is smooth and somewhat thickened with respect to the cylinder oil but is still fluid.

According to the present invention, the use of the amic acid derivatives produces a substantially more uniform grease base. It is true that there may be some variation in the content of the amines employed to produce the amic acids, but in general it is possible to secure amines and other constituents which are approximately 98% pure and we prefer to use such compounds in making up our greases and other compounds in order to avoid the difficulties encountered in the use of natural fats and fatty acids as heretofore employed. The salts of amic acid prepared by us in accordance with our invention include the following:

(B)



where X is an alkali metal, and R, R<sub>1</sub> and R<sub>2</sub> are as above defined.

(C)



where M is an alkaline earth metal; R, R<sub>1</sub> and R<sub>2</sub> are as above defined, and R<sub>3</sub> is selected from the group consisting of hydrogen and an amic acid radical having the formula

(D)



where R, R<sub>1</sub> and R<sub>2</sub> are as above defined, and R<sub>3</sub> and R<sub>4</sub> are each selected from the group consisting of hydrogen and an amic acid radical having the formula



The substances prepared by us in accordance with our invention may be either condensations of a primary amine with a dibasic acid or they may be condensations of a secondary amine with a dibasic acid. For example but without limitation, as indicated below, we have produced in accordance with our invention, N-mono-lauryl adipamic acid prepared from a primary amine, and N-di-lauryl adipamic acid prepared from a secondary amine. It is not necessary, of course, that the radicals, R<sub>1</sub> and R<sub>2</sub>, as given in the above formulae, should be identical. They may be the same or they may be radicals of different chain lengths within the definitions given therewith. Thus, we recognize compounds such as N-lauryl-palmityl-adipamic acid and similar substituted acids where R<sub>1</sub> and R<sub>2</sub> are of different chain lengths as falling under the formulae above given.

The amic acids of our invention result from the condensation of an amine with a dibasic acid in stoichiometrical proportions so as to amide only one of the available carboxyl groups in accordance with the following general equations:

(E)



(F)



where R, R<sub>1</sub> and R<sub>2</sub> are as hereinabove defined.

We may employ in accordance with our invention the following dibasic acids falling under the above Formula E: Itaconic acid, adipic acid (hexanedioic acid), succinic acid (butanedioic acid), azelaic acid (nonanedioic acid), sebacic acid (decanedioic acid), and malonic acid (propanedioic acid), and others.

Illustrative of the amines which may be either primary or secondary amines are the following: Mono-n-butylamine, mono-n-hexylamine, mono-n-octylamine, mono-n-decylamine, mono-laurylamine, mono-myristylamine, mono-palmitylamine, mono-stearylamine, mono-linoleylamine, mono-oleylamine, di-octylamine, di-laurylamine, di-palmitylamine and di-stearylamine. These amines, as procurable, may contain a mixture of amines, which will react and appear in the final product. Thus, lauryl amine may contain small quantities of other amines such as octylamine, but we prefer to keep the quantity of such impurities limited to a small amount.

The following are examples illustrative of our invention of (I) Amic acids, (II) Salts of such acids and greases made therefrom, and (III) Mixed amic acids and greases therefrom; including processes for making each of Groups I, II and III. It is to be understood that these examples together with the examples of the dibasic acids and amines given above are illustrative and the invention is not to be considered as limited thereto except as indicated in the appended claims.

The molecular weights of the amic acids which are given below as theoretical are the molecular weights calculated from the reacting weights of the commercial ingredients which as heretofore stated may contain small amounts of impurities. To the extent that these impurities occur, the stated theoretical molecular weights of the compounds differ from the theoretical molecular weights of compounds of 100% purity.

#### (I) AMIC ACIDS

##### 1. N-mono-n-butyl-sebacamic acid

|    |                                                                                                                                                                                 |             |
|----|---------------------------------------------------------------------------------------------------------------------------------------------------------------------------------|-------------|
| 45 | $\begin{array}{c} \text{O} \quad \text{O} \quad \text{H} \\ \parallel \quad \parallel \\ \text{HO}-\text{C}-(\text{CH}_2)_8-\text{C}-\text{N}-\text{C}_2\text{H}_5 \end{array}$ | Parts       |
|    | Mono-n-butylamine                                                                                                                                                               | 73 (26.4%)  |
| 50 | Sebacic acid                                                                                                                                                                    | 203 (73.6%) |

The sebacic acid was heated to its melting point (approximately 270° F.). The butylamine was added slowly, with no agitation, the temperature being permitted to rise to 290-310° F. after all of the amine had been added. After two (2) hours at 290-310° F., acidity checking revealed the end of the reaction. The loss in weight, as water, was determined as a cross-check on the end point of the reaction.

| 60                               | Test Data | Theoretical | Actual |
|----------------------------------|-----------|-------------|--------|
| Water loss                       | percent   | 6.53        | 6.61   |
| Acidity—calculated as oleic acid | do        | 109.3       | 110.0  |
| Melting point                    | °C        |             | 80.0   |
| Nitrogen                         | percent   | 5.43        | 5.38   |
| Mean molecular weight            |           | 258         | 256.1  |
| Color                            |           |             | White  |
| Odor                             |           |             | Bland  |

##### 2. N-mono-n-octyl-sebacamic acid

|    |                                                                                                                                                                                    |              |
|----|------------------------------------------------------------------------------------------------------------------------------------------------------------------------------------|--------------|
| 70 | $\begin{array}{c} \text{O} \quad \text{O} \quad \text{H} \\ \parallel \quad \parallel \\ \text{HO}-\text{C}-(\text{CH}_2)_8-\text{C}-\text{N}-\text{C}_8\text{H}_{17} \end{array}$ | Parts        |
|    | Mono-n-octylamine                                                                                                                                                                  | 129 (38.85%) |
| 75 | Sebacic acid                                                                                                                                                                       | 203 (61.15%) |

The process was carried out as in Example 1, but the reaction was complete in 2½ hours, as indicated by the acidity test.

| Test Data                               | Theoretical | Actual |
|-----------------------------------------|-------------|--------|
| Water loss.....percent                  | 5.42        | 5.60   |
| Acidity—calculated as oleic acid.....do | 89.80       | 89.95  |
| Melting point.....°C                    | 88.9        | 88.9   |
| Nitrogen.....percent                    | 4.46        | 4.41   |
| Mean molecular weight                   | 314         | 313.8  |
| Color                                   | White       |        |
| Odor                                    | Bland       |        |

### 3. N-mono-decyl-sebacamic acid



Parts  
Decylamine 157 (43.6%)  
Sebacic acid 203 (56.4%)

The batch was processed as for Example 1, except that the reaction time was three (3) hours.

| Test Data                               | Theoretical | Actual |
|-----------------------------------------|-------------|--------|
| Water loss.....percent                  | 5.0         | 5.2    |
| Acidity—calculated as oleic acid.....do | 82.4        | 82.9   |
| Melting point.....°C                    | 94.5        | 94.5   |
| Nitrogen.....percent                    | 4.09        | 3.98   |
| Mean molecular weight                   | 342         | 340    |
| Color                                   | White       |        |
| Odor                                    | Spicy       |        |

### 4. N-mono-lauryl-sebacamic acid



Parts  
Laurylamine 185 (47.7%)  
Sebacic acid 203 (52.3%)

The batch was processed as for Example 1, except that the reaction time was four (4) hours.

| Test Data                               | Theoretical | Actual |
|-----------------------------------------|-------------|--------|
| Water loss.....percent                  | 4.64        | 4.70   |
| Acidity—calculated as oleic acid.....do | 76.2        | 76.7   |
| Melting point.....°C                    | 98.5        | 98.5   |
| Nitrogen.....percent                    | 3.78        | 3.70   |
| Mean molecular weight                   | 370         | 368    |
| Color                                   | White       |        |
| Odor                                    | Spicy       |        |

### 5. N-mono-myristyl-sebacamic acid



Parts  
Myristylamine 213 (51.2%)  
Sebacic acid 203 (48.8%)

The batch was made up exactly as for Example 4.

| Test Data                               | Theoretical | Actual |
|-----------------------------------------|-------------|--------|
| Water loss.....percent                  | 4.33        | 4.41   |
| Acidity—calculated as oleic acid.....do | 70.8        | 71.3   |
| Melting point.....°C                    | 103.5       | 103.5  |
| Nitrogen.....percent                    | 3.51        | 3.47   |
| Mean molecular weight                   | 398         | 395    |
| Color                                   | White       |        |
| Odor                                    | Spicy       |        |

### 6. N-mono-palmityl-sebacamic acid



Parts  
Palmitylamine 242 (54.3%)  
Sebacic acid 203 (45.7%)

The batch was made up exactly as for Example 4.

| Test Data                               | Theoretical | Actual |
|-----------------------------------------|-------------|--------|
| Water loss.....percent                  | 4.05        | 4.20   |
| Acidity—calculated as oleic acid.....do | 66.1        | 66.6   |
| Melting point.....°C                    | 109.0       |        |
| Nitrogen.....percent                    | 3.28        | 3.22   |
| Mean molecular weight                   | 427         | 424    |
| Color                                   | White       |        |
| Odor                                    | Spicy       |        |

### 7. N-mono-stearyl-sebacamic acid



Parts  
Mono-stearylamine 270 (57%)  
Sebacic acid 203 (43%)

The batch was processed as for Example 1, except that the reaction time was 5½ hours.

| Test Data                               | Theoretical | Actual |
|-----------------------------------------|-------------|--------|
| Water loss.....percent                  | 3.8         | 3.95   |
| Acidity—calculated as oleic acid.....do | 61.9        | 62.0   |
| Melting point.....°C                    | 114.5       |        |
| Nitrogen.....percent                    | 3.07        | 3.01   |
| Mean molecular weight                   | 455         | 454    |
| Color                                   | White       |        |
| Odor                                    | Spicy       |        |

### 8. N-mono-oleyl-sebacamic acid



Parts  
Mono-oleylamine 268 (56.8%)  
Sebacic acid 203 (43.2%)

The batch was processed exactly as for Example 4.

| Test Data                               | Theoretical  | Actual |
|-----------------------------------------|--------------|--------|
| Water loss.....percent                  | 3.82         | 3.90   |
| Acidity—calculated as oleic acid.....do | 62.2         | 62.7   |
| Melting point.....°C                    | 99.2         |        |
| Nitrogen.....percent                    | 3.08         | 3.06   |
| Mean molecular weight                   | 453          | 450    |
| Color                                   | Golden Brown |        |
| Odor                                    | Spicy        |        |

### 9. N-dilauryl-sebacamic acid



Parts  
Sec. laurylamine 356 (63.7%)  
Sebacic acid 203 (36.3%)

The batch was processed as for Example 1, except that the reaction time was six (6) hours.

| Test Data                               | Theoretical | Actual |
|-----------------------------------------|-------------|--------|
| Water loss.....percent                  | 3.22        | 3.18   |
| Acidity—calculated as oleic acid.....do | 62.2        | 62.4   |
| Melting point.....°C                    | 81.1        |        |
| Nitrogen.....percent                    | 2.59        | 2.56   |
| Mean molecular weight                   | 541         | 538    |
| Color                                   | Tan         |        |
| Odor                                    | Soapy       |        |

### 10. N-dipalmityl-sebacamic acid



Parts  
Sec. palmitylamine 465 (69.6%)  
Sebacic acid 203 (30.4%)

The batch was processed exactly as for Example 9.

| Test data                                    | Theoretical | Actual |
|----------------------------------------------|-------------|--------|
| Water loss.....percent.....                  | 2.69        | 2.63   |
| Acidity—calculated as oleic acid.....do..... | 43.4        | 43.7   |
| Melting point.....°C.....                    | 87.6        | 87.7   |
| Nitrogen.....percent.....                    | 2.15        | 2.12   |
| Mean molecular weight.....                   | 650         | 645    |
| Color.....                                   | Cream       |        |
| Odor.....                                    | Bland       |        |

11. *N*-distearyl-sebacamic acid



| Parts                              |
|------------------------------------|
| Sec. stearylamine..... 521 (71.9%) |
| Sebacic acid..... 203 (28.1%)      |

The batch was made exactly as in Example 9.

| Test Data                                    | Theoretical | Actual |
|----------------------------------------------|-------------|--------|
| Water loss.....percent.....                  | 2.49        | 2.44   |
| Acidity—calculated as oleic acid.....do..... | 40.0        | 40.3   |
| Melting point.....°C.....                    | 89.5        | 89.5   |
| Nitrogen.....percent.....                    | 1.98        | 1.92   |
| Mean molecular weight.....                   | 706         | 700    |
| Color.....                                   | Cream       |        |
| Odor.....                                    | Bland       |        |

12. *N*-mono-*n*-butyl-azelaamic acid



| Parts                                      |
|--------------------------------------------|
| Mono- <i>n</i> -butylamine..... 73 (27.8%) |
| Azelaic acid..... 190 (72.2%)              |

The batch was processed exactly as in Example 1.

| Test Data                                    | Theoretical | Actual  |
|----------------------------------------------|-------------|---------|
| Water loss.....percent.....                  | 6.34        | 6.30    |
| Acidity—calculated as oleic acid.....do..... | 115.0       | 115.4   |
| Melting point.....°C.....                    | 22          | 22      |
| Nitrogen.....percent.....                    | 5.72        | 5.68    |
| Mean molecular weight.....                   | 245         | 244.2   |
| Color.....                                   | Amber       | viscous |
| Odor.....                                    | fluid       | Bland   |

13. *N*-mono-*n*-hexyl-azelaamic acid



| Parts                                       |
|---------------------------------------------|
| Mono- <i>n</i> -hexylamine..... 101 (34.7%) |
| Azelaic acid..... 190 (65.3%)               |

The batch was processed exactly as in Example 1.

| Test Data                                    | Theoretical | Actual |
|----------------------------------------------|-------------|--------|
| Water loss.....percent.....                  | 6.19        | 6.24   |
| Acidity—calculated as oleic acid.....do..... | 104.0       | 103.7  |
| Melting point.....°C.....                    | 21          | 21     |
| Nitrogen.....percent.....                    | 5.07        | 5.12   |
| Mean molecular weight.....                   | 271         | 271.5  |
| Color.....                                   | White       |        |
| Odor.....                                    | Spicy       |        |

14. *N*-mono-*n*-octyl-azelaamic acid



| Parts                                       |
|---------------------------------------------|
| Mono- <i>n</i> -octylamine..... 130 (40.7%) |
| Azelaic acid..... 190 (59.3%)               |

The batch was processed exactly as in Example 3.

| Test Data                                    | Theoretical | Actual |
|----------------------------------------------|-------------|--------|
| Water loss.....percent.....                  | 5.62        | 5.57   |
| Acidity—calculated as oleic acid.....do..... | 93.3        | 84.3   |
| Melting point.....°C.....                    |             |        |
| Nitrogen.....percent.....                    | 4.64        | 4.59   |
| Mean molecular weight.....                   | 302         | 301    |
| Color.....                                   | White       |        |
| Odor.....                                    | Spicy       |        |

15. *N*-mono decyl-azelaamic acid



| Parts                                        |
|----------------------------------------------|
| Mono- <i>n</i> -decylamine ..... 160 (45.7%) |
| Azelaic acid ..... 190 (54.3%)               |

The batch was processed exactly as in Example 3.

| Test Data                                    | Theoretical | Actual |
|----------------------------------------------|-------------|--------|
| Water loss.....percent.....                  | 5.14        | 5.0    |
| Acidity—calculated as oleic acid.....do..... | 84.9        | 85.7   |
| Melting point.....°C.....                    |             |        |
| Nitrogen.....percent.....                    | 4.22        | 4.14   |
| Mean molecular weight.....                   | 332         | 331    |
| Color.....                                   | Cream       |        |
| Odor.....                                    | Spicy       |        |

16. *N*-mono lauryl-azelaamic acid



| Parts                             |
|-----------------------------------|
| Monolaurylamine ..... 188 (49.8%) |
| Azelaic acid ..... 190 (50.2%)    |

The batch was processed exactly as in Example 4.

| Test Data                                    | Theoretical | Actual |
|----------------------------------------------|-------------|--------|
| Water loss.....percent.....                  | 4.77        | 4.78   |
| Acidity—calculated as oleic acid.....do..... | 78.3        | 78.5   |
| Melting point.....°C.....                    |             |        |
| Nitrogen.....percent.....                    | 3.89        | 3.83   |
| Mean molecular weight.....                   | 360         | 359    |
| Color.....                                   | Light Brown |        |
| Odor.....                                    | Spicy       |        |

17. *N*-mono myristyl-azelaamic acid



| Parts                               |
|-------------------------------------|
| Monomyristylamine ..... 215 (53.2%) |
| Azelaic acid ..... 190 (46.8%)      |

The batch was processed exactly as in Example 4.

| Test Data                                    | Theoretical | Actual |
|----------------------------------------------|-------------|--------|
| Water loss.....percent.....                  | 4.45        | 4.49   |
| Acidity—calculated as oleic acid.....do..... | 72.8        | 73.1   |
| Melting point.....°C.....                    |             |        |
| Nitrogen.....percent.....                    | 3.61        | 3.55   |
| Mean molecular weight.....                   | 387         | 385.5  |
| Color.....                                   | Cream       |        |
| Odor.....                                    | Bland       |        |

18. *N*-mono palmityl-azelaamic acid



| Parts                               |
|-------------------------------------|
| Monopalmitylamine ..... 245 (56.3%) |
| Azelaic acid ..... 190 (43.7%)      |

The batch was processed as in Example 1, except that the reaction time was four and one-half (4½) hours.

| Test Data                                    | Theoretical | Actual |
|----------------------------------------------|-------------|--------|
| Water loss.....percent.....                  | 4.14        | 4.02   |
| Acidity—calculated as oleic acid.....do..... | 67.7        | 67.9   |
| Melting point.....°C.....                    | 91.2        | 91.2   |
| Nitrogen.....percent.....                    | 3.36        | 3.40   |
| Mean molecular weight.....                   | 417         | 415    |
| Color.....                                   | Cream       |        |
| Odor.....                                    | Bland       |        |

19. *N*-mono stearyl-azelaämic acid



Parts

|                        |             |
|------------------------|-------------|
| Monostearylamine ..... | 270 (58.7%) |
| Azelaic acid.....      | 190 (41.3%) |

The batch was processed exactly as in Example 7.

| Test Data                                    | Theoretical | Actual |
|----------------------------------------------|-------------|--------|
| Water loss.....percent.....                  | 3.02        | 3.87   |
| Acidity—calculated as oleic acid.....do..... | 63.9        | 64.2   |
| Melting point.....°C.....                    | 105.0       |        |
| Nitrogen.....percent.....                    | 3.17        | 3.11   |
| Mean molecular weight.....                   | 452         | 440    |
| Color.....                                   | Light Brown |        |
| Odor.....                                    | Spicy       |        |

20. *N*-mono oleyl-azelaämic acid



Parts

|                      |             |
|----------------------|-------------|
| Monooleylamine ..... | 267 (58.3%) |
| Azelaic acid.....    | 190 (41.7%) |

The batch was processed exactly as in Example 4.

| Test Data                                    | Theoretical | Actual |
|----------------------------------------------|-------------|--------|
| Water loss.....percent.....                  | 3.94        | 3.86   |
| Acidity—calculated as oleic acid.....do..... | 64.2        | 64.5   |
| Melting point.....°C.....                    | 78.2        |        |
| Nitrogen.....percent.....                    | 3.19        | 3.20   |
| Mean molecular weight.....                   | 439         | 437    |
| Color.....                                   | Deep amber  |        |
| Odor.....                                    | Spicy       |        |

21. *N*-dilauryl-azelaämic acid



Parts

|                        |             |
|------------------------|-------------|
| Sec. laurylamine ..... | 356 (65.2%) |
| Azelaic acid.....      | 190 (34.8%) |

The batch was processed as in Example 9.

| Test Data                                    | Theoretical | Actual |
|----------------------------------------------|-------------|--------|
| Water loss.....percent.....                  | 3.30        | 3.24   |
| Acidity—calculated as oleic acid.....do..... | 53.3        | 53.7   |
| Melting point.....°C.....                    | 70.6        |        |
| Nitrogen.....percent.....                    | 2.65        | 2.59   |
| Mean molecular weight.....                   | 528         | 525    |
| Color.....                                   | Brown       |        |
| Odor.....                                    | Soapy       |        |

22. *N*-dipalmityl-azelaämic acid



Parts

|                          |             |
|--------------------------|-------------|
| Sec. palmitylamine ..... | 465 (71.0%) |
| Azelaic acid.....        | 190 (29.0%) |

The batch was processed as in Example 9.

| Test Data                                    | Theoretical | Actual |
|----------------------------------------------|-------------|--------|
| Water loss.....per cent.....                 | 2.75        | 2.79   |
| Acidity—calculated as oleic acid.....do..... | 44.3        | 44.5   |
| Melting point.....°C.....                    | 72.4        |        |
| Nitrogen.....per cent.....                   | 2.20        | 2.17   |
| Mean molecular weight.....                   | 637         | 634    |
| Color.....                                   | Tan         |        |
| Odor.....                                    | Bland       |        |

23. *N*-distearyl-azelaämic acid



| Parts                              |
|------------------------------------|
| Sec. stearylamine..... 521 (73.3%) |
| Adipic acid..... 190 (26.7%)       |

The batch was made exactly as in Example 9.

| Test Data                                    | Theoretical | Actual |
|----------------------------------------------|-------------|--------|
| Water loss.....per cent.....                 | 2.53        | 2.60   |
| Acidity—calculated as oleic acid.....do..... | 40.7        | 40.9   |
| Melting point.....°C.....                    | 76.6        |        |
| Nitrogen.....per cent.....                   | 2.02        | 2.00   |
| Mean molecular weight.....                   | 693         | 690    |
| Color.....                                   | Tan         |        |
| Odor.....                                    | Bland       |        |

24. *N*-mono-*n*-butyl-adipamic acid



Parts

|                                     |             |
|-------------------------------------|-------------|
| 35 Mono- <i>n</i> -butylamine ..... | 73 (33.1%)  |
| Adipic acid.....                    | 148 (66.9%) |

The batch was processed exactly as in Example 1.

| Test Data                                    | Theoretical | Actual |
|----------------------------------------------|-------------|--------|
| Water loss.....per cent.....                 | 8.15        | 8.01   |
| Acidity—calculated as oleic acid.....do..... | 139.0       | 139.6  |
| Melting point.....°C.....                    | 93.3        |        |
| Nitrogen.....per cent.....                   | 6.89        | 6.80   |
| Mean molecular weight.....                   | 203         | 202    |
| Color.....                                   | White       |        |
| Odor.....                                    | Bland       |        |

25. *N*-mono-*n*-hexyl-adipamic acid



Parts

|                                     |             |
|-------------------------------------|-------------|
| 55 Mono- <i>n</i> -hexylamine ..... | 101 (40.6%) |
| Adipic acid.....                    | 148 (59.4%) |

The batch was made exactly as in Example 1.

| Test Data                                    | Theoretical | Actual |
|----------------------------------------------|-------------|--------|
| Water loss.....per cent.....                 | 7.23        | 7.33   |
| Acidity—calculated as oleic acid.....do..... | 122.0       | 122.4  |
| Melting point.....°C.....                    | 104.7       |        |
| Nitrogen.....per cent.....                   | 6.06        | 5.94   |
| Mean molecular weight.....                   | 231         | 230    |
| Color.....                                   | White       |        |
| Odor.....                                    | Spicy       |        |

26. *N*-mono-*n*-octyl-adipamic acid



Parts

|                                     |             |
|-------------------------------------|-------------|
| 70 Mono- <i>n</i> -octylamine ..... | 130 (46.8%) |
| Adipic acid.....                    | 148 (53.2%) |

11

The batch was made exactly as in Example 3.

| Test Data                                    | Theoretical | Actual |
|----------------------------------------------|-------------|--------|
| Water loss.....per cent.....                 | 6.48        | 6.52   |
| Acidity—calculated as oleic acid.....do..... | 108.3       | 108.7  |
| Melting point.....°C.....                    | 115.6       | 115.6  |
| Nitrogen.....per cent.....                   | 5.38        | 5.30   |
| Mean molecular weight.....                   | 260         | 259    |
| Color.....                                   | White       |        |
| Odor.....                                    | Spicy       |        |

27. *N*-mono decyl-adipamic acid

Parts

|                          |             |
|--------------------------|-------------|
| Mono-n-decyllamine ..... | 160 (51.9%) |
| Adipic acid.....         | 148 (48.1%) |

The batch was processed exactly as in Example 3.

| Test Data                                    | Theoretical | Actual |
|----------------------------------------------|-------------|--------|
| Water loss.....per cent.....                 | 5.84        | 5.92   |
| Acidity—calculated as oleic acid.....do..... | 97.3        | 97.7   |
| Melting point.....°C.....                    | 105.0       | 105.0  |
| Nitrogen.....per cent.....                   | 4.83        | 4.77   |
| Mean molecular weight.....                   | 290         | 288.5  |
| Color.....                                   | White       |        |
| Odor.....                                    | Spicy       |        |

28. *N*-monolauryl-adipamic acid

Parts

|                    |             |
|--------------------|-------------|
| Lauryllamine ..... | 188 (55.9%) |
| Adipic acid.....   | 148 (44.1%) |

The batch was processed exactly as in Example 4.

| Test Data                                    | Theoretical | Actual |
|----------------------------------------------|-------------|--------|
| Water loss.....Per Cent.....                 | 5.36        | 5.42   |
| Acidity—calculated as oleic acid.....do..... | 88.7        | 89.0   |
| Melting point.....°C.....                    | 96.7        | 96.7   |
| Nitrogen.....Per Cent.....                   | 4.40        | 4.42   |
| Mean molecular weight.....                   | 318         | 316.5  |
| Color.....                                   | White       |        |
| Odor.....                                    | Spicy       |        |

29. *N*-monomyristyl-adipamic acid

Parts

|                     |             |
|---------------------|-------------|
| Myristylamine ..... | 215 (59.2%) |
| Adipic acid.....    | 148 (40.8%) |

The batch was processed exactly as in Example 4.

| Test Data                                    | Theoretical | Actual |
|----------------------------------------------|-------------|--------|
| Water loss.....Per Cent.....                 | 4.96        | 5.01   |
| Acidity—calculated as oleic acid.....do..... | 81.7        | 81.9   |
| Melton point.....°C.....                     | 89.0        | 89.0   |
| Nitrogen.....Per Cent.....                   | 4.06        | 3.94   |
| Mean molecular weight.....                   | 345         | 344    |
| Color.....                                   | White       |        |
| Odor.....                                    | Bland       |        |

30. *N*-monopalmityl-adipamic acid

Parts

|                     |             |
|---------------------|-------------|
| Palmitylamine ..... | 245 (62.4%) |
| Adipic acid.....    | 148 (37.6%) |

12

The batch was processed exactly as in Example 4.

| Test Data                                    | Theoretical | Actual |
|----------------------------------------------|-------------|--------|
| Water loss.....Percent.....                  | 4.58        | 4.63   |
| Acidity—calculated as oleic acid.....do..... | 75.2        | 75.5   |
| Melting point.....°C.....                    | 82.0        | 82.0   |
| Nitrogen.....percent.....                    | 3.73        | 3.70   |
| Mean molecular weight.....                   | 375         | 373    |
| Color.....                                   | White       |        |
| Odor.....                                    | Bland       |        |

31. *N*-monostearyl-adipamic acid

| Test Data                                    | Theoretical | Actual |
|----------------------------------------------|-------------|--------|
| Water loss.....Percent.....                  | 4.31        | 4.41   |
| Acidity—calculated as oleic acid.....do..... | 70.5        | 70.7   |
| Melting point.....°C.....                    | 81.4        | 81.4   |
| Nitrogen.....percent.....                    | 3.50        | 3.47   |
| Mean molecular weight.....                   | 400         | 399    |
| Color.....                                   | Tan         |        |
| Odor.....                                    | Bland       |        |

The batch was processed exactly as in Example 7.

| Test Data                                    | Theoretical | Actual |
|----------------------------------------------|-------------|--------|
| Water loss.....Percent.....                  | 4.31        | 4.41   |
| Acidity—calculated as oleic acid.....do..... | 70.5        | 70.7   |
| Melting point.....°C.....                    | 81.4        | 81.4   |
| Nitrogen.....percent.....                    | 3.50        | 3.47   |
| Mean molecular weight.....                   | 400         | 399    |
| Color.....                                   | Tan         |        |
| Odor.....                                    | Bland       |        |

32. *N*-monooleyl-adipamic acid

| Test Data                                    | Theoretical | Actual |
|----------------------------------------------|-------------|--------|
| Water loss.....Percent.....                  | 4.34        | 4.50   |
| Acidity—calculated as oleic acid.....do..... | 71.0        | 71.3   |
| Melting point.....°C.....                    | 76.2        | 76.2   |
| Nitrogen.....percent.....                    | 3.53        | 3.50   |
| Mean molecular weight.....                   | 397         | 396    |
| Color.....                                   | Opaque      |        |
| Odor.....                                    | Amber       |        |

The batch was processed exactly as in Example 7.

| Test Data                                    | Theoretical | Actual |
|----------------------------------------------|-------------|--------|
| Water loss.....Percent.....                  | 4.34        | 4.50   |
| Acidity—calculated as oleic acid.....do..... | 71.0        | 71.3   |
| Melting point.....°C.....                    | 76.2        | 76.2   |
| Nitrogen.....percent.....                    | 3.53        | 3.50   |
| Mean molecular weight.....                   | 397         | 396    |
| Color.....                                   | Opaque      |        |
| Odor.....                                    | Amber       |        |

33. *N*-dilauryl-adipamic acid

| Test Data                                    | Theoretical | Actual |
|----------------------------------------------|-------------|--------|
| Water loss.....Percent.....                  | 4.34        | 4.50   |
| Acidity—calculated as oleic acid.....do..... | 71.0        | 71.3   |
| Melting point.....°C.....                    | 76.2        | 76.2   |
| Nitrogen.....percent.....                    | 3.53        | 3.50   |
| Mean molecular weight.....                   | 397         | 396    |
| Color.....                                   | Opaque      |        |
| Odor.....                                    | Amber       |        |

The batch was processed exactly as in Example 9.

| Test Data                                    | Theoretical | Actual |
|----------------------------------------------|-------------|--------|
| Water loss.....Percent.....                  | 3.57        | 3.61   |
| Acidity—calculated as oleic acid.....do..... | 53.0        | 53.3   |
| Melting point.....°C.....                    | 81.1        | 81.1   |
| Nitrogen.....percent.....                    | 2.88        | 2.81   |
| Mean molecular weight.....                   | 486         | 484    |
| Color.....                                   | Tan         |        |
| Odor.....                                    | Soapy       |        |

34. *N*-dipalmityl-adipamic acid

| Test Data                                    | Theoretical | Actual |
|----------------------------------------------|-------------|--------|
| Water loss.....Percent.....                  | 465         | 75.8%  |
| Acidity—calculated as oleic acid.....do..... | 148         | 24.2%  |
| Melting point.....°C.....                    |             |        |
| Nitrogen.....percent.....                    |             |        |
| Mean molecular weight.....                   |             |        |
| Color.....                                   |             |        |
| Odor.....                                    |             |        |



15

by cessation of evolution of water, after forty (40) minutes.

| Test Data                           | Theoretical | Actual |
|-------------------------------------|-------------|--------|
| Water loss percent                  | 8.87        | 9.15   |
| Acidity—calculated as oleic acid do | 152.5       | 153.0  |
| Melting point °C                    | (1)         |        |
| Nitrogen percent                    | 7.56        | 7.53   |
| Mean molecular weight               | 185         | 184    |
| Color                               | Straw       |        |
| Odor                                | Bland       | 10     |

<sup>1</sup> Viscous liquid with -11° C. freezing point.

41. *N*-mono-*n*-octyl-itaconamic acid



|                            | Parts    |
|----------------------------|----------|
| Mono- <i>n</i> -octylamine | 130(50%) |
| Itaconic acid              | 130(50%) |

The batch was made as in Example 40, except that the reaction time was one (1) hour.

| Test Data                           | Theoretical | Actual |
|-------------------------------------|-------------|--------|
| Water loss percent                  | 6.93        | 6.99   |
| Acidity—calculated as oleic acid do | 116.5       | 116.9  |
| Melting point °C                    | 34.4        | 34.4   |
| Nitrogen percent                    | 5.78        | 57.1   |
| Mean molecular weight               | 242         | 241    |
| Color                               | Yellow      |        |
| Odor                                | Spicy       | 35     |

42. *N*-mono-decyl-itaconamic acid



|                | Parts      |
|----------------|------------|
| Monodecylamine | 160(55.2%) |
| Itaconic acid  | 130(44.8%) |

The batch was processed as in Example 40, except that the reaction time was 80 minutes.

| Test Data                           | Theoretical | Actual |
|-------------------------------------|-------------|--------|
| Water loss percent                  | 6.21        | 6.40   |
| Acidity—calculated as oleic acid do | 103.7       | 104.0  |
| Melting point °C                    | 36.7        | 5.11   |
| Nitrogen percent                    | 5.15        | 271.5  |
| Mean molecular weight               | 272         | Yellow |
| Color                               |             | Spicy  |
| Odor                                |             | 60     |

43. *N*-mono lauryl-itaconamic acid



|                  | Parts      |
|------------------|------------|
| Mono laurylamine | 188(59.2%) |
| Itaconic acid    | 130(40.8%) |

16

The batch was made exactly as in Example 42.

|    | Test Data                           | Theoretical | Actual |
|----|-------------------------------------|-------------|--------|
| 5  | Water loss percent                  | 5.66        | 5.71   |
|    | Acidity—calculated as oleic acid do | 94.0        | 94.3   |
| 10 | Melting point °C                    | 40.0        |        |
|    | Nitrogen percent                    | 4.67        | 4.64   |
| 15 | Mean molecular weight               | 300         | 299    |
|    | Color                               |             | Cream  |
| 20 | Odor                                |             | Spicy  |

44. *N*-monomyristyl-itaconamic acid



|               | Parts      |
|---------------|------------|
| Myristylamine | 215(62.3%) |
| Itaconic acid | 130(37.7%) |

The batch was made exactly as in Example 42.

|    | Test Data                           | Theoretical | Actual |
|----|-------------------------------------|-------------|--------|
| 30 | Water loss percent                  | 5.22        | 5.40   |
|    | Acidity—calculated as oleic acid do | 86.2        | 86.4   |
| 35 | Melting point °C                    | 48.7        |        |
|    | Nitrogen percent                    | 4.28        | 4.22   |
| 40 | Mean molecular weight               | 327         | 326    |
|    | Color                               |             | Cream  |
| 45 | Odor                                |             | Spicy  |

45. *N*-mono palmityl-itaconamic acid



|                    | Parts      |
|--------------------|------------|
| Mono palmitylamine | 245(65.3%) |
| Itaconic acid      | 130(34.7%) |

The batch was made exactly as in Example 42.

|    | Test Data                           | Theoretical | Actual |
|----|-------------------------------------|-------------|--------|
| 55 | Water loss percent                  | 4.8         | 5.1    |
|    | Acidity—calculated as oleic acid do | 79.0        | 79.7   |
| 60 | Melting point °C                    | 59.2        |        |
|    | Nitrogen percent                    | 3.92        | 3.87   |
| 65 | Mean molecular weight               | 357         | 354    |
|    | Color                               |             | Cream  |
| 70 | Odor                                |             | Spicy  |

46. *N*-mono stearyl-itaconamic acid



|                   | Parts      |
|-------------------|------------|
| Mono stearylamine | 270(67.5%) |
| Itaconic acid     | 130(32.5%) |

17

The batch was processed the same as in Example 42, except that the reaction time was two (2) hours.

| Test Data                             | Theoretical | Actual |
|---------------------------------------|-------------|--------|
| Water loss.....                       | percent     | 4.5    |
| Acidity—calculated as oleic acid..... | do          | 73.8   |
| Melting point.....                    | ° C         | 68.6   |
| Nitrogen.....                         | percent     | 3.67   |
| Mean molecular weight.....            |             | 382    |
| Color.....                            |             | Tan    |
| Odor.....                             |             | Spicy  |

**(II) SALTS OF SUCH ACIDS AND GREASES MADE THEREFROM**

The alkali, alkaline earth, and other polyvalent metal salts of the above amic acids are employed with oils to form greases in accordance with our invention. Below are listed examples of products utilizing the above types of ingredients.

**47. *N-lauryl-sodium sebacamate grease***



|                                            | Per cent |
|--------------------------------------------|----------|
| N-lauryl sebacamate acid.....              | 10       |
| Sodium hydroxide—flake.....                | 1        |
| 200/100° F. S. S. U. Coastal pale oil..... | 89       |
|                                            | 100      |
| Salt content.....                          | 10.6     |

The N-lauryl sebacamic acid and oil are added to a kettle and heated to about 400–440° F. The sodium hydroxide is dissolved in three times its weight of water and is slowly added to the heated sebacamic acid and oil in the kettle. Reaction commences. The addition of the alkali solution is controlled so that the temperature is about 435° F. when all of the alkali has been completely added; the grease is cooled to about 120° F. maximum without disturbing, that is, without raking, stirring or otherwise agitating it. The grease is then milled, that is, passed over rollers, kettle stirred, or passed through a homogenizer or mill until the structure is substantially homogeneous.

The above grease had the following properties:

|                                                                          |         |
|--------------------------------------------------------------------------|---------|
| Penetration ASTM (American Society for Testing Materials) D-217-47T..... | 296     |
| Dropping point (D.P.) ASTM-566-42.....                                   | 379° F. |
| Water tolerance Chrysler.....                                            | 10%     |
| Color.....                                                               | Straw   |

**48. *N-lauryl-lithium sebacamate grease***



|                                            | Per cent |
|--------------------------------------------|----------|
| N-lauryl-sebacamic acid.....               | 10       |
| Lithium hydroxide monohydrate.....         | 1        |
| 100/100° F. S. S. U. Coastal pale oil..... | 89       |
|                                            | 100      |
| Salt content.....                          | 10.13    |

The batch was made exactly as in Example 47. The finished grease had the following properties:

|                                 |               |
|---------------------------------|---------------|
| Penetration ASTM D-217-47T..... | 320           |
| D./P. ASTM D-566-42.....        | 409° F.       |
| Water tolerance Chrysler.....   | Less than 10% |

18

**49. *N-lauryl-lithium sebacamate grease***

|                                               | Per cent |
|-----------------------------------------------|----------|
| N-lauryl-sebacamic acid.....                  | 10       |
| Lithium hydroxide monohydrate.....            | 1        |
| 3500/100° F. S. S. U. Residual black oil..... | 89       |

100  
Salt content..... 10.13

10 The batch was made exactly as in Example 47. The finished grease had the following properties:

|                                         |                      |
|-----------------------------------------|----------------------|
| Penetration ASTM D-217-47T.....         | 288                  |
| D./P. ASTM D-566-42.....                | 410° F.              |
| C. R. C. wheel bearing grease test..... | Fair to good         |
| Rust prevention—10% salt spray.....     | O. K. after 72 hours |

**50. *N-lauryl-barium sebacamate grease***

|                                                           | Per cent |
|-----------------------------------------------------------|----------|
| N-lauryl-sebacamic acid.....                              | 11.44    |
| Barium hydroxide octahydrate.....                         | 4.28     |
| 200/210° F. S. S. U. Mid-Continent semi-bright stock..... | 84.28    |
|                                                           | 100.00   |

Salt content..... 13.25

35 The batch was made exactly as in Example 47 except that crystals of alkali were used. The finished grease had the following properties:

|                                         |         |
|-----------------------------------------|---------|
| Penetration ASTM D-217-47T.....         | 295     |
| D./P. ASTM D-566-42.....                | 355° F. |
| C. R. C. wheel bearing grease test..... | Good    |

Water tolerance Chrysler..... Less than 10%

**51. *N-lauryl-calcium sebacamate grease***

|                                                           | Per cent |
|-----------------------------------------------------------|----------|
| N-lauryl-sebacamic acid.....                              | 10       |
| Calcium hydroxide—100% 200-mesh.....                      | 1        |
| 200/210° F. S. S. U. Mid-Continent semi-bright stock..... | 89       |
|                                                           | 100      |

55 Salt content..... 10.62

The batch was processed as in Example 47, except that the lime was made up as a 1:3 slurry in oil. The finished grease had the following properties:

|                                 |         |
|---------------------------------|---------|
| Penetration ASTM D-217-47T..... | 298     |
| D./P. ASTM D-566-42.....        | 294° F. |

**52. *N-lauryl-strontium sebacamate grease***

|                                               | Per cent |
|-----------------------------------------------|----------|
| N-lauryl sebacamic acid.....                  | 10.0     |
| Strontium hydroxide octahydrate.....          | 3.1      |
| 3500/100° F. S. S. U. Residual black oil..... | 86.9     |
|                                               | 100.0    |

75 Salt content..... 11.05

19

The batch was processed as in Example 50. The finished grease had the following properties:

Penetration ASTM D-217-47T ..... 311  
D./P. ASTM D-566-42 ..... 310° F.  
5 53. *N-lauryl-lithium sebacamate grease*

Per cent  
N-lauryl sebacamic acid ..... 10  
Lithium hydroxide monohydrate ..... 1  
100/100° F. S. S. U. solvent extracted Mid-  
Continent pale oil ..... 89  
100  
15 Salt content ..... 10.13

The batch was made exactly as in Example 47. The finished grease had the following properties:

Penetration ASTM D-217-47T ..... 332  
D./P. ASTM D-566-42 ..... 396° F.  
20 54. *N-oleyl-lithium sebacamate grease*

Per cent  
N-oleyl-sebacamic acid ..... 10  
Lithium hydroxide monohydrate ..... .75  
100/100° F. Coastal pale oil ..... 89.25  
100.00  
15 Salt content ..... 10.02

The batch was made as in Example 47. The finished grease had the following properties:

Penetration ASTM D-217-47T ..... 316  
D./P. ASTM D-566-42 ..... 405° F.  
35 55. *N-oleyl-lithium sebacamate grease*

Per cent  
N-oleyl-sebacamic acid ..... 10  
Lithium hydroxide monohydrate ..... .75  
300/100° F. S. S. U. Tech. white oil ..... 89.25  
100.00  
15 Salt content ..... 10.02

The batch was made as in Example 47. The finished grease had the following properties:

Penetration ASTM D-217-47T ..... 327  
D./P. ASTM D-566-42 ..... 395° F.  
40 56. *N-lauryl-sodium sebacamate grease*

Per cent  
N-lauryl-sebacamic acid ..... 10  
Sodium hydroxide ..... 1  
100/100° F. S. S. U. Coastal pale oil ..... 89  
100  
15 Salt content ..... 10.6

The batch was made as in Example 47. The finished grease had the following properties:

Penetration ASTM D-217-47T ..... 270  
D./P. ASTM D-566-42 ..... 360° F.  
45 57. *N-lauryl-lithium sebacamate grease*

Per cent  
N-oleyl-sebacamic acid ..... 10  
Lithium hydroxide monohydrate ..... 1  
200/100° F. S. S. U. Mid-Continent pale  
oil ..... 44.5  
180/210° F. S. S. U. Mid-Continent bright  
stock ..... 44.5  
100.00  
15 Salt content ..... 10.13

20

The batch was made as in Example 47. The finished grease had the following properties:

Penetration ASTM D-217-47T ..... 298  
D./P. ASTM D-566-42 ..... 427° F.  
5 Water tolerance Chrysler ..... 10%

58. *N-lauryl-sodium sebacamate grease*  
Per cent  
N-lauryl-sebacamic acid ..... 15.00  
10 Sodium hydroxide ..... 1.50  
180/210° F. S. S. U. Mid-Continent bright  
stock ..... 41.75  
200/100° F. S. S. U. Mid-Continent pale  
oil ..... 41.75  
15 Salt content ..... 100.00

Salt content ..... 15.9

The batch was made as in Example 47. The finished grease had the following properties:

20 Penetration ASTM D-217-47T ..... 245  
D./P. ASTM D-566-42 ..... °F. 375  
Water tolerance Chrysler ..... per cent 65

59. *N-palmityl-lithium sebacamate grease*  
Per cent  
N-palmityl-sebacamic acid ..... 10.0  
30 Lithium hydroxide monohydrate ..... 0.9  
3500/100° F. S. S. U. Residual black oil ..... 89.1  
100.00  
15 Salt content ..... 10.16

The batch was made as in Example 47. The finished grease had the following properties:

Penetration ASTM D-217-47T ..... 240  
D./P. ASTM D-566-42 ..... °F. 410  
60 60. *N-palmityl-sodium sebacamate grease*

Per cent  
N-palmityl-sebacamic acid ..... 10.0  
45 Sodium hydroxide ..... 0.9  
3500/100° F. S. S. U. Residual black oil ..... 89.1  
100.00  
15 Salt content ..... 10.51

The batch was made as in Example 47. The finished grease had the following properties:

Penetration ASTM D-217-47T ..... 245  
D./P. ASTM D-566-42 ..... °F. 371  
55 61. *N-palmityl-sodium sebacamate grease*

The grease of Example 60 was diluted further with Residual black oil 3500/100° F. S. S. U. at room temperature so that the salt content in the formula was about 2.9%. The properties of this composition were:

Penetration ASTM D-217-47T ..... 406  
Dropping point ASTM D-566-42 ..... °F. 367  
65 62. *N-lauryl-sodium azelaämate grease*

Per cent  
N-lauryl-azelaämic acid ..... 6  
70 Sodium hydroxide ..... 0.67  
300/100° F. S. S. U. Coastal pale oil ..... 93.33  
100.00  
15 Salt content ..... 6.42

## 21

The batch was made as in Example 47. The finished grease had the following properties:

Penetration ASTM D-217-47T 341  
D./P. ASTM D-566-42 345 °F.

63. *N-lauryl-lithium azelaämate grease*

Per cent 10

N-lauryl-azelaämic acid 6  
Lithium hydroxide monohydrate 0.67  
300/100° F. S. S. U. Coastal pale oil 93.33

100.00 15

Salt content 6.1

The batch was made as in Example 47. The finished grease had the following properties:

Penetration ASTM D-217-47T 330 20  
D./P. ASTM D-566-42 395 °F.

64. *N-lauryl-lithium sebacamate grease*

Per cent 25

N-lauryl-sebacamic acid 4.0  
Lithium hydroxide monohydrate 0.4  
150/210° F. S. S. U. Residual black oil 57.3

100/100° F. S. S. U. Coastal pale oil 38.3

100.00 30

Salt content 4.05

The batch was made as in Example 47. The finished grease had the following properties:

Penetration ASTM D-217-47T 348 348  
D./P. ASTM D-566-42 395 °F.

65. *N-stearyl lithium itaconamate grease*

Per cent

N-stearyl-itaconamic acid 10.0  
Lithium hydroxide monohydrate 1.1  
75/210° F. S. S. U. Mid-Continent bright

stock 88.9

100.00 45

Salt content 10.23

The batch was made as in Example 47. The finished grease had the following properties:

Penetration ASTM D-217-47T 340 55  
D./P. ASTM D-566-42 370 °F.

66. *N-decyl-lithium adipamate grease*

Per cent

N-decyl-adipamic acid 10.0  
Lithium hydroxide monohydrate 1.45  
75/210° F. S. S. U. Mid-Continent bright

stock 88.55

100.00 65

Salt content 9.46

The batch was made as in Example 47. The finished grease had the following properties:

Penetration ASTM D-217-47T 326 70  
D./P. ASTM D-566-42 391 °F.

## 22

67. *N-dilauryl-lithium adipamate grease*

Per cent

N-dilauryl-adipamic acid 10.0  
Lithium hydroxide monohydrate 0.87  
300/100° F. Mid-Continent pale oil 89.13

100.00

Salt content 10.21

The batch was made as in Example 47. The finished grease had the following properties:

Penetration ASTM D-217-47T 310 20  
D./P. ASTM D-566-42 411 °F.

C. R. C. wheel bearing grease test Good

68. *N-stearyl-lithium azelaämate grease*

Per cent

N-stearyl-azelaämic acid 10.0  
Lithium hydroxide monohydrate 0.93  
75/210° F. Coastal bright stock 89.07

100.00

Salt content 10.2

The batch was made as in Example 47. The finished grease had the following properties:

Penetration ASTM D-217-47T 295 20  
D./P. ASTM D-566-42 416 °F.

69. *N-butyl-lithium sebacamate grease*

Per cent

N-butyl-sebacamic acid 10.0  
Lithium hydroxide monohydrate 1.63  
600/100° F. Mid-Continent lube distil-  
late 88.37

100.00

Salt content 10.38

The batch was made as in Example 47. The finished grease had the following properties:

Penetration ASTM D-217-47T 316 20  
D./P. ASTM D-566-42 394 °F.

70. *N-oleyl-lithium sebacamate grease*

Per cent

N-oleyl sebacamic acid 1.0  
Lithium hydroxide monohydrate 0.09  
100/100° F. S. S. U. Coastal pale oil 8.9  
300/100° F. S. S. U. Coastal pale oil 90.01

100.00

Salt content 1.02

The batch was made as in Example 47. The finished grease was fluid and had the following properties:

Viscosity (Gardiner Mobiometer at  
77° F.)<sup>1</sup> 1-100-1000  
Pour point °F. -15

<sup>1</sup> This test is made with a series of disks numbered from 1 to 3 with arbitrary weights, the viscosity being measured by disk movement through the material tested and being represented in seconds.

The above Gardner Mobilometer viscosity is designated as "1-100-1000" which represents #1 disk, 100 gm. weight, and 1000 seconds at 77° F. Gardner Mobilometer viscosities hereinafter referred to are simply designated similarly to the expression quoted above.

71. *N-lauryl-lithium sebacamate grease*

|                                   | Per cent |
|-----------------------------------|----------|
| N-lauryl-sebacamic acid           | 30       |
| Lithium hydroxide monohydrate     | 2.3      |
| 300/100° F. Mid-Continent neutral | 67.7     |
|                                   | 100.0    |
| Salt content                      | 30.39    |
|                                   | 15       |

The batch was made as in Example 47. The finished grease had the following properties:

|                            |         |
|----------------------------|---------|
| Penetration ASTM D-217-47T | 107     |
| D./P. ASTM D-566-42        | °F. 471 |
| Water tolerance Chrysler   | Nil     |

72. *N-lauryl-potassium sebacamate grease*

|                                          | Per cent |
|------------------------------------------|----------|
| N-lauryl-sebacamic acid                  | 10.0     |
| Potassium hydroxide                      | 1.5      |
| 75/210° F. S. S. U. Coastal bright stock | 88.5     |
|                                          | 100.0    |
| Salt content                             | 11.06    |

The batch was made as in Example 47. The finished grease had the following properties:

|                            |             |
|----------------------------|-------------|
| Penetration ASTM D-217-47T | 342         |
| D./P. ASTM D-566-42        | °F. 379     |
| Water tolerance Chrysler   | per cent 30 |

73. *N-lauryl-lithium sebacamate grease*

|                                             | Per cent |
|---------------------------------------------|----------|
| N-lauryl-sebacamic acid                     | 10       |
| Lithium hydroxide                           | 1        |
| 180/210° F. S. S. U. Coastal cylinder stock | 87       |
| Lead naphthenate (30% lead)                 | 2        |
|                                             | 100      |
| Salt content                                | 10.13    |

The 180/210° F. S. S. U. Coastal cylinder stock and N-lauryl sebacamic acid were heated to 400° F. with constant agitation. After the acid had completely melted and dispersed in the oil, the neutralization with the lithium hydroxide (15-20%) solution in water was begun. The neutralization was carried out and the grease processed, without lead naphthenate, as described in Example 47.

After the grease had cooled to room temperature, it was melted to a smooth, homogeneous consistency, after which the lead naphthenate was added and blended in. It must be noted that the lead naphthenate should not be included in the high temperature phase operation in this grease formulation.

The physical properties of the resultant grease were:

|                                       |             |
|---------------------------------------|-------------|
| Penetration—unworked                  | 245         |
| Penetration ASTM D-217-47T            | 280         |
| Penetration—5000 strokes              | 320         |
| D./P. ASTM D-566-42                   | °F. 405     |
| Chrysler basket D./P.                 | °F. 330     |
| Water tolerance Chrysler              | per cent 10 |
| Rust preventive test (10% salt spray) |             |
| O. K. after 72 hours                  | 75          |

74. *N-lauryl-lithium sebacamate grease*

|                                             | Per cent |
|---------------------------------------------|----------|
| N-lauryl-sebacamic acid                     | 5.0      |
| Lithium hydroxide monohydrate               | 0.5      |
| 180/210° F. S. S. U. Coastal cylinder stock | 92.5     |
| Lead naphthenate (30% lead)                 | 2.0      |
|                                             | 100.0    |

|              |      |
|--------------|------|
| Salt content | 5.06 |
|--------------|------|

The batch was made exactly as in Example 73. The physical properties of the resultant grease were:

|                            |             |
|----------------------------|-------------|
| Penetration—unworked       | 302         |
| Penetration ASTM D-217-47T | 304         |
| Penetration—5000 strokes   | 346         |
| D./P. ASTM D-566-42        | °F. 397     |
| Chrysler basket D./P.      | °F. 310     |
| Water tolerance Chrysler   | per cent 10 |

75. *N-lauryl-lithium sebacamate grease*

|                                       | Per cent |
|---------------------------------------|----------|
| N-lauryl-sebacamic acid               | 2.0      |
| Lithium hydroxide monohydrate         | 0.2      |
| Sulfurized lard oil (10% sulfur)      | 10.0     |
| 300/100° F. S. S. U. Coastal pale oil | 87.8     |
|                                       | 100.0    |
| Salt content                          | 2.05     |

It is to be noted that due to the sulfur in the sulfurized lard oil, that material can not be included in the high temperature operation in the manufacture of these greases, so that the N-lauryl sebacamic acid and the mineral oil are heated to 400° F. and processed as in Example 47.

After the grease had been melted to a homogeneous mass, the sulfurized lard oil was blended into the grease.

The resultant grease had the following properties:

|                                           |                       |
|-------------------------------------------|-----------------------|
| Viscosity (Gardner Mobilometer at 77° F.) | 2-50-(40 to 50)       |
| Almen test carries                        | 20 lb. lever arm load |
| Falex test (500 lb. step test)            | 3000 lbs. gauge       |
| Falex test (100 lb. step test)            | 2700 lbs. gauge       |
| Water tolerance Chrysler                  | 10%                   |
| Heat stability test:                      |                       |

Since the material is wholly fluid, standard dropping points as a measurement of heat or temperature resistance could not be applied. In this case, then, Gardner Mobilometer tests were run at varying temperatures:

|                           |            |
|---------------------------|------------|
| At 77° F. actual run was  | 43 seconds |
| At 100° F. actual run was | 42 seconds |
| At 125° F. actual run was | 42 seconds |
| At 150° F. actual run was | 40 seconds |
| At 200° F. actual run was | 40 seconds |

## 25

76. *N-lauryl-lithium sebacamate grease*

|                                             | Per cent |
|---------------------------------------------|----------|
| N-lauryl sebacamic acid                     | 0.5      |
| Lithium hydroxide monohydrate               | 0.05     |
| 180/210° F. S. S. U. Coastal cylinder stock | 69.60    |
| 100/100° F. S. S. U. Coastal pale oil       | 29.85    |
|                                             | 100.00   |

Salt content 5

The batch was made as in Example 47. The resultant grease had the following properties:

Viscosity (Gardner Mobilometer at 77° F.) 2-50-(30 to 40)

Water tolerance Chrysler 10%

Heat stability test (Gardner Mobilometer):

|                           |            |
|---------------------------|------------|
| At 77° F. actual run was  | 36 seconds |
| At 100° F. actual run was | 36 seconds |
| At 125° F. actual run was | 40 seconds |
| At 150° F. actual run was | 39 seconds |
| At 200° F. actual run was | 39 seconds |

Rust preventive test (10% salt spray) O. K. after 72 hrs.

The heat stability test indicated that the grease does not thin out rapidly as the temperature is elevated under ordinary operating conditions.

77. *Aluminum-mono-N-lauryl sebacamate grease*

392 parts of the sodium salt of the N-lauryl sebacamic acid were dissolved in 1000 parts of water at room temperature. To this solution were added 80 parts of sodium hydroxide. When the above solution was homogeneous, it was heated to boiling, about 212° F. A solution made up of 171 parts of aluminum sulfate nonahydrate dissolved in 500 parts of water was slowly added to the first solution. Boiling was maintained and, after all of the solution had been added, the boiling was continued for 30 minutes. The salt which had risen to the top of the aqueous portion was separated from the aqueous portion by siphoning off the aqueous portion. Fresh water was added to the salt and reboiled. This separation and reboiling was continued with fresh water until the aqueous portion was neutral to phenolphthalein. The salt was then dried and powdered.

A mixture of the aluminum salt and oil to make the grease was prepared in the following manner:

|                                       | Per cent |
|---------------------------------------|----------|
| Aluminum mono-N-lauryl sebacamate     | 10       |
| 300/100° F. S. S. U. Coastal pale oil | 90       |
|                                       | 100      |

The powdered aluminum mono-N-lauryl sebacamate was mixed into the oil to make a pasty slurry. The mass was heated, with continuous agitation to the point where the mass turned from a pasty mass to a clear solution (about 375° F.). The mass was permitted to cool to room temperature without agitation. When cool, the grease was milled out to a homogeneous mass. The finished grease had the following properties:

Penetration ASTM D-217-47T 346

D./P. ASTM D-566-42 °F. 316

Water tolerance Chrysler per cent 25

75

## 26

78. *Aluminum-di-N-lauryl sebacamate grease*

To 392 parts of sodium N-lauryl sebacamate (prepared as hereinbelow, Example 80) dissolved in 1000 parts of water was added 126 parts of aluminum sulfate nonahydrate dissolved in 500 parts of water. The mass was heated to boiling. The precipitate formed was purified by subsequent washings with boiling distilled water until washings were neutral to phenolphthalein. The washed precipitate was dried and powdered.

A mixture of the aluminum salt and oil to make the grease was prepared in the following manner:

|                                             | Per cent |
|---------------------------------------------|----------|
| Aluminum di-N-lauryl sebacamate             | 10       |
| 300/100° F. S. S. U. Mid-Continent pale oil | 90       |
|                                             | 100      |

The powdered aluminum di-N-lauryl sebacamate and the oil were mixed in a kettle to a pasty consistency and were then gradually heated to about 440° F. with continuous agitation. The mass changes from a pasty opaque mass to a transparent fluid after heating for about 20 minutes. The mass was allowed to cool to room temperature without agitation. When cool, the mass was milled out smooth by agitating in the kettle. The resulting product was a smooth, adhesive, transparent grease. The grease had the following properties:

|    |                                                       |
|----|-------------------------------------------------------|
| 35 | Penetration ASTM D-217-47T 310                        |
| 36 | D./P. ASTM D-566-42 394° F.                           |
| 37 | Water tolerance Chrysler 15%                          |
| 40 | Color Golden Yellow                                   |
| 41 | C. R. C. wheel bearing grease test Fair               |
| 42 | Rust preventive (10% salt spray) O. K. after 72 hours |

79. *Aluminum tri-N-oleyl adipamate grease*

420 parts of sodium N-oleyl adipamate (prepared as hereinbelow, Example 80) were dissolved in 1000 parts of water and the whole was brought to a boil. To the hot salt solution was slowly added the hot solution of 57 parts of aluminum sulfate nonahydrate in 300 parts of water. Since there were three (3) parts of sodium salt in excess, the reaction mixture was alkaline to phenolphthalein. The aluminum salt was purified by several washings of boiling water, until the washings were neutral to phenolphthalein. The salt was then dried and powdered.

A mixture of the aluminum salt and oil to make the grease was prepared in the following manner:

|                                       | Per cent |
|---------------------------------------|----------|
| Aluminum N-oleyl adipamate            | 10       |
| 300/100° F. S. S. U. Coastal pale oil | 90       |
|                                       | 100      |

The mixture was processed as in Example 77. The finished grease had the following properties:

Penetration ASTM D-217-47T 330

D./P. ASTM D-366-42 °F. 344

Water tolerance Chrysler per cent 15

The following procedure was used to make the sodium salts of the amic acids in their separate form. These sodium salts were used in the preparation of the aluminum salts above.

80. *Process for making alkali metal and alkaline earth metal salts of amic acids*



370 parts of the N-lauryl sebacamic acid were dissolved in 1000 parts of ethanol. To this alcoholic solution was added, dropwise, an alcoholic solution of 40 parts of sodium hydroxide in 300 parts of ethanol. This was insufficient alkali to give color indication with phenolphthalein so a slight excess of 2 parts of NaOH in 15 parts of alcohol was added and was found sufficient to give the phenolphthalein color test. The phenolphthalein color indication was just discharged by introduction of carbon dioxide gas into the solution. Then the alcohol was distilled off, and the anhydrous salt (sodium N-lauryl sebacamate) was pulverized at  $-10^{\circ}\text{ F}$ .

A similar process to the above may be employed for producing the other alkali metal salts of the various amic acids.

The alkaline earth metal salts of the various amic acids may be made in a similar manner to the aluminum salts made above, namely, by combining the alkali metal salt of the amic acid in water solution with the appropriate alkaline earth chloride or other water-soluble alkaline earth salt. Purification is accomplished in the same manner as stated for the aluminum salts above.

(III) MIXED AMIC ACIDS AND GREASES THEREFROM

It has been found in accordance with our invention that by using mixtures of one or more different salts of amic acids, we may vary the properties thereof and of the greases therefrom advantageously. For example, but without limitation, we may improve the water tolerance characteristic of a grease by using a grease ingredient having an exceptional water tolerance, such as but without limitation, a salt of N-stearyl sebacamic acid; or rust protection may be improved by using a salt of N-oleyl sebacamic acid; or shear stability may be improved by using a salt of N-lauryl sebacamic acid; or dropping point may be improved by using a salt of N-octyl sebacamic acid. These various salts of amic acids mentioned in this paragraph may be combined with one another or with other herein mentioned amic acid salts to give the properties desired.

We have found that there are available commercially certain amines which contain varying proportions of primary and secondary amines.

Illustrative of the mixed amines, but without limitation, is a technical lauryl amine of the following constituency:

|                        | Per cent   |
|------------------------|------------|
| Primary amines         | 85         |
| Octyl amine            | per cent 8 |
| Decyl amine            | do 9       |
| Dodecyl (lauryl) amine | do 47      |
| Tetradecylamine        | do 18      |
| Hexadecylamine         | do 8       |
| Octadecylamine         | do 5       |
| Octadecenylamine       | do 5       |
| Mixed secondary amines | 15         |

This mixed amine will produce, of course, a mixture of the corresponding amic acids with the dibasic acid selected.

By test, it was determined that the reacting (equivalent) weight of the technical lauryl amine is 235. This weight was then used in determining the reaction mixtures of the acid and amine in the preparation of amic acids as follows:

81. *N-Tech. lauryl-adipamic acid*



mixed with



and other like compounds of different hydrocarbon chain lengths in the amine group.

|                   | Parts       |
|-------------------|-------------|
| Tech. laurylamine | 235 (61.7%) |
| Adipic acid       | 146 (38.3%) |

The amic acid was made in the same way as provided in Example 4.

The amic acid had the following properties:

|                                  | Test Data | Theoretical | Actual |
|----------------------------------|-----------|-------------|--------|
| 30 Yield                         | percent   | 95.3        | 94.9   |
| Water loss                       | do        | 4.7         | 5.1    |
| Nitrogen                         | do        | 3.86        | 3.80   |
| Mean molecular weight            |           | 363         | 365    |
| Acidity—calculated as oleic acid | percent   | 77.7        | 77.38  |
| Melting point                    | °C        |             | 124    |
| Appearance                       |           |             | (1)    |
| Odor                             |           |             | Soapy  |

<sup>1</sup> Amorphous creamy white solid.

82. *N-Tech. lauryl-sebacamic acid*



mixed with



and other like compounds of different hydrocarbon chain lengths in the amine group.

|                   | Parts       |
|-------------------|-------------|
| Tech. laurylamine | 235 (53.6%) |
| Sebacic acid      | 203 (46.4%) |

The amic acid was made in the same way as provided in Example 4.

The amic acid had the following properties:

|                                     | Test Data | Theoretical | Actual  |
|-------------------------------------|-----------|-------------|---------|
| 55 Yield                            | percent   | 95.8        | 95.6    |
| Water loss                          | do        | 4.2         | 4.4     |
| Nitrogen                            | do        | 3.33        | 3.29    |
| 60 Acidity—calculated as oleic acid | percent   | 67.2        | 67.4    |
| Mean molecular weight               |           | 420         | 418     |
| Melting point                       |           |             | 109° C. |
| Appearance                          |           |             | (1)     |
| Odor                                |           |             | Soapy   |

<sup>1</sup> Light tan amorphous solid.

83. *Lithium-N-Tech. lauryl sebacamate grease*



mixed with



and other like compounds of different hydrocarbon chain lengths in the amine group.

Per cent  
 N-Tech. lauryl sebacamic acid 10  
 Lithium hydroxide monohydrate 1  
 600/100° F. S. S. U. Coastal cylinder oil  
 blend 39.5

100  
 Salt content 10.2

The batch was made exactly as in Example 47.  
 The finished grease had the following properties:

Penetration ASTM D-217-47T 276  
 Penetration—unworked 276  
 Penetration—5000 strokes 324  
 D.P. ASTM D-566-42 416° F.  
 Chrysler basket D.P. 367° F.  
 Water tolerance Chrysler 15%  
 C. R. C. wheel bearing grease test O. K.  
 Rust preventive (10% salt spray) O. K. after 72 hours  
 G. E. ball bearing test (212° F. at 3450 R. P. M.) O. K. after 200 hours, no sign of failure

The properties represent a combination of properties resulting from the use of the mixture of amines in the formation of the grease base, which accordingly is a mixture of salts of the various amic acids made from such amines.

Lubricating greases made with compounds in accordance with our invention are superior to the greases made with the natural fatty materials in that the dropping points of the greases made in accordance with our invention are from 50-75° F. higher than the best natural fat greases of equivalent gelator content. Also, the amic acid compound greases, because of the polarity of the gelator are rust preventives and will actually displace water from metal surfaces, and will resist water after the surface has once been treated with the lubricant. In addition, natural fatty materials are mixtures of substances, some of which do not form greases. These non-grease forming substances are present in varying amounts and accordingly change the greases. In the greases of our invention all ingredients employed form greases and there is substantially no non-grease forming material.

When properly compounded, our amic acid compound greases can be used at operating temperatures much nearer their ASTM dropping points than can the natural fat greases of equivalent gelator content.

The resistance to shear of our amic acid greases is much greater than the natural fat greases of equivalent gelator content.

The control of the manufacture of the greases of our invention is easier than in the manufacture of natural fat greases.

What we claim is:

1. As a new composition, a mixture containing a substantial proportion of a gelation agent and a petroleum lubricant, said gelation agent being selected from the group consisting of the alkali metal salt of an amic acid having the formula



and a polyvalent metal salt of said amic acid, where R is selected from the group consisting of methylene groups having a carbon chain length of 1 to 8 carbon atoms and the group



R<sub>1</sub> is an aliphatic radical of a carbon chain length of 4 to 18 carbon atoms, and R<sub>2</sub> is selected from the group consisting of hydrogen and an aliphatic radical of a carbon chain length of 4 to 18 carbon atoms.

2. As a new composition, a mixture containing a substantial proportion of a gelation agent and a petroleum lubricant, said gelation agent being a compound having the formula



where X is an alkali metal, R is selected from the group consisting of methylene groups having a carbon chain length of 1 to 8 carbon atoms and the group



20 R<sub>1</sub> is an aliphatic radical of a carbon chain length of 4 to 18 carbon atoms, and R<sub>2</sub> is selected from the group consisting of hydrogen and an aliphatic radical of a carbon chain length of 4 to 18 carbon atoms.

25 3. As a new composition, a mixture containing a substantial proportion of a gelation agent and a petroleum lubricant, said gelation agent being a compound having the formula



where M is an alkaline earth metal; R is selected from the group consisting of methylene groups having a carbon chain of 1 to 8 carbon atoms and the group



40 R<sub>2</sub> is an aliphatic radical of a carbon chain length of 4 to 18 carbon atoms, and R<sub>3</sub> is selected from the group consisting of hydrogen and an amic acid radical having the formula



45 4. As a new composition, a mixture containing a substantial proportion of a gelation agent and a petroleum lubricant, said gelation agent being a compound having the formula



55 where R is selected from the group consisting of methylene groups having a carbon chain of 1 to 8 carbon atoms and the group



60 R<sub>1</sub> is an aliphatic radical of a carbon chain length of 4 to 18 carbon atoms; R<sub>2</sub> is selected from the group consisting of hydrogen and an aliphatic radical of a carbon chain length of 4 to 18 carbon atoms, and R<sub>3</sub> and R<sub>4</sub> are each selected from the group consisting of hydrogen and an amic acid radical having the formula



65 5. A grease having about 0.5% to 30% grease base of the total weight of the grease, said grease base being selected from the group consisting of

## 31

an alkali metal salt and a polyvalent metal salt of an amic acid having the formula



where R is selected from the group consisting of methylene groups having a carbon chain length of 1 to 8 carbon atoms and the group



R<sub>1</sub> is an aliphatic radical of a carbon chain length of 4 to 18 carbon atoms, and R<sub>2</sub> is selected from the group consisting of hydrogen and an aliphatic radical of a carbon chain length of 4 to 18 carbon atoms, and the remainder of the grease being composed principally of petroleum oil.

6. A grease having about 6 to about 17% of grease base, said grease base being selected from the group consisting of an alkali metal salt and a polyvalent metal salt of an amic acid having the formula



where R is selected from the group consisting of methylene groups having a carbon chain length of 1 to 8 carbon atoms and the group



R<sub>1</sub> is an aliphatic radical of a carbon chain length of 4 to 18 carbon atoms, and R<sub>2</sub> is selected from the group consisting of hydrogen and an aliphatic radical of a carbon chain length of 4 to 18 carbon atoms, and the remainder of the grease being composed principally of petroleum oil.

7. A grease composed of about 0.5 to 30% of N-lauryl.alkali metal sebacamate and the remainder being composed substantially of mineral oil.

8. A grease composed of about 10 to 13% of N-lauryl.alkaline earth metal sebacamate and the remainder being composed substantially of mineral oil.

9. A grease composed of about 1 to 10% of N-oleyl.alkali metal sebacamate and the remainder being composed substantially of mineral oil.

10. A grease composed of about 10% of N-palmityl.alkali metal sebacamate and the remainder being composed substantially of mineral oil.

11. A grease composed of about 6% of N-lauryl.alkali metal azelaämate, and the remainder being composed substantially of mineral oil.

12. A grease composed of about 10% of aluminum di-N-lauryl sebacamate and the remainder being composed substantially of mineral oil.

13. A composition containing a substantial proportion of a gelation agent and a petroleum lubricant, said gelation agent being a mixture of at

## 32

least two substances selected from the group consisting of the alkali metal salt of an amic acid having the formula



and a polyvalent metal salt of said amic acid, where R is selected from the group consisting of methylene groups having a carbon chain length of 1 to 8 carbon atoms and the group



R<sub>1</sub> is an aliphatic radical of a carbon chain length of 4 to 18 carbon atoms, and R is selected from the group consisting of hydrogen and an aliphatic radical of a carbon chain length of 4 to 18 carbon atoms.

14. A composition containing a substantial proportion of a gelation agent and a petroleum lubricant, said gelation agent being a mixture of at least two substances selected from the group consisting of an amic acid salt having the formula



where X is an alkali metal, R is selected from the group consisting of methylene groups having a carbon chain length of 1 to 8 carbon atoms and the group



R<sub>1</sub> is an aliphatic radical of a carbon chain length of 4 to 18 carbon atoms, and R<sub>2</sub> is selected from the group consisting of hydrogen and an aliphatic radical of a carbon chain length of 4 to 18 carbon atoms, the difference between the substances of the mixture being constituted by a different chain length in the aliphatic radicals attached to the N atom.

WILLIAM C. BRYANT.  
ANTHONY GIORDANO.

## REFERENCES CITED

The following references are of record in the file of this patent:

## UNITED STATES PATENTS

| Number       | Name              | Date          |
|--------------|-------------------|---------------|
| 50 2,191,738 | Balle             | Feb. 27, 1940 |
| 2,191,978    | Balle et al.      | Feb. 27, 1940 |
| 2,283,602    | Fiero             | May 19, 1942  |
| 2,322,783    | Katzman et al.    | June 29, 1943 |
| 2,324,712    | Lynch             | July 20, 1943 |
| 55 2,363,510 | Farrington et al. | Nov. 28, 1944 |
| 2,378,442    | Smith et al.      | June 19, 1945 |
| 2,378,443    | Smith et al.      | June 19, 1945 |
| 2,432,049    | Swan et al.       | Dec. 2, 1947  |
| 2,458,425    | Rocchini          | Jan. 4, 1949  |
| 2,480,743    | Krantz et al.     | Aug. 30, 1949 |